

Nov. 13, 1934.

S. P. LOVELL

1,980,810

SHOE STIFFENER

Filed June 25, 1932



Inventor  
Stanley P. Lovell  
By Knight, Brown, Dunlap & May

Attest:

## UNITED STATES PATENT OFFICE

1,980,810

## SHOE STIFFENER

Stanley P. Lovell, Newton, Mass., assignor to  
Arden Box Toe Company, Watertown, Mass., a  
corporation of Massachusetts

Application June 25, 1932, Serial No. 619,296

11 Claims. (Cl. 154—46)

The subject of this invention is shoe stiffener parts, and more especially those known as box toes and intended to maintain the shape, as well as to impart such qualities as strength, resilience, and water resistance to the fore part of a shoe.

In realizing a box toe of the desired strength and resilience and yet possessed of the proper thinness, it is sometimes the practice to build up a laminated structure whose plies consist of suitable fabric, e. g., textile fabric or paper felt carrying a suitable stiffening agent. For instance, the plies may carry a coating of celluloid or other cellulose ester capable of being gelatinized by a suitable solvent, so as to permit the stiffener blank to acquire the plastic or mouldable state requisite for incorporation into and shaping with the shoe upper during the pulling-over and lasting operations. When such a stiffener undergoes solvent treatment, the cellulose ester in the coating tends to migrate into the fabric and to lose itself, so to speak, in the fabric fibers, with a consequent loss in stiffness. Under the stress of lasting, this tendency is increased; and the gelatinized cellulose is apt to ooze at the edges 25 of the superposed stiffener plies.

In accordance with the present invention, I construct a laminated stiffener comprising a fabric ply charged with a suitable stiffening agent and united to a preformed, substantially continuous film of suitable cellulose ester. The fabric ply may be paper felt, woven textile fabric, or the like. The stiffening agent in the fabric may be a compound similar to or different from the compound constituting the preformed film, but it should be capable of being gelatinized by a solvent of the preformed film of cellulose ester. The preferred form of stiffener is one made up of at least three superposed, united plies, the inner ply of which is the preformed film of cellulose ester, and the outer plies of which are fabric charged with the appropriate stiffening agent. Such a stiffener has the qualities of stiffness and resiliency to a high degree, by virtue of the fact that when it is exposed to solvent action preparatory to assembly with a shoe upper, as by momentary immersion in a solvent bath, the preformed film is not rendered entirely fluid and the stiffener as a whole imbibes comparatively little solvent and hence exhibits a high ratio of stiffening solids to solvent. In other words, the preformed film, rather than being dissolved and dissipated, merely undergoes incipient solution on its surfaces, wherefore it simply becomes tenaciously integrated with the fabric plies whose stiffening agent 55 has undergone more or less complete gelatiniza-

tion by solvent action. The preformed film thus exists in the moulded and assembled stiffener in a condition to augment most effectively the stiffness and resiliency furnished by the stiffened fabric plies. In making the stiffener, I may die out blanks of the proper shape from the preformed film and from the stiffened fabric, and unite them in superposed relationship under the influence of solvent action. For instance, assuming that a fabric has been stiffened by impregnation with a solution of cellulose ester, stiffener blanks may be died out from the fabric while it is still sufficiently wet with the solution to permit bonding with similar blanks cut from the preformed film. Should the impregnated fabric be dried before cutting into blanks, the blanks may be moistened with solvent on their surfaces to be bonded with the blanks of preformed film. Or, if desired, whole sheets of impregnated fabric may be bonded face to face with whole sheets of preformed film, and the resulting laminated structure then died out into shoe stiffener blanks. In making a three-ply stiffener, for example, it is possible to feed a sheet of the preformed film in between two sheets of freshly impregnated fabric proceeding from the impregnating baths in a properly squeezed condition. The three-ply structure may be fed into press rolls to ensure the desired union between the plies, then dried, and cut into the stiffener blanks.

On the accompanying drawing,

Figure 1 illustrates a two-ply stiffener embodying the present invention and whose fabric ply is lifted from the preformed, substantially continuous film.

Figure 2 similarly illustrates a three-ply stiffener.

Figure 3 depicts a stiffener made up with a still larger number of plies and whose thickness is shown greatly enlarged.

The stiffener shown in Figure 1 is a box toe and consists of a preformed, substantially continuous film of cellulose ester bonded to a fabric ply charged with a stiffening agent capable of being gelatinized by a solvent of the particular cellulose ester constituting the film. In fact, the stiffening agent for the fabric may be a cellulose ester similar to that of the film. It is preferable, however, that two stiffened fabric plies be combined with an internal stiffening phase of preformed film. A box toe is shown so constructed, in Figure 2, with cellulose acetate as the stiffening agent in both the film and fabric plies. When more than three plies are used, as in the stiffener illustrated in Figure 3, the stiffened fabric inner

- plies may well be of the nature of paper felt, and the stiffened outer fabric plies be a woven or similar textile fabric. The outer plies may be of the same size, whereas the internal laminae 5 may consist of alternate blanks of stiffened paper and preformed film progressively decreasing in size from one outer ply to the other. This means that the stiffener will terminate, as shown, in comparatively thin beveled edges or margins, which 10 comport with comfort and smoothness in the finished shoe. A similar effect may be had by skiving a stiffener, all of whose constituent plies are of the same size, at its marginal or edge portions.
- 15 It is inevitable that the amount of stiffening agent per unit of volume is lower in the fabric plies than in the preformed film, as the stiffening agent merely occupies pores and interstices in the fabric, whereas the film consists entirely of stiffening agent. I prefer that the stiffened fabric have a porosity permissive of a quick penetration of the solvent therethrough, so as to reach the film of cellulose ester, even though this means that the fabric will not be charged with a saturating 20 amount of stiffening agent and thus be stiffened short of its potential limit. Let us consider, for example, a three-ply stiffener made in accordance with the present invention and intended to be used in women's street shoes. Such a stiffener 25 may comprise outer fabric plies, such as napped cotton twill, of a thickness of approximately .018 inch and carrying as an impregnant, say, 2½ to 3 ounces of cellulose ester per square yard, and an inner, preformed film of cellulose ester of 30 a thickness of only .003 inch and weighing as much as the upper limit of cellulose ester content in the fabric, namely, 3 ounces per square yard. When the cellulose ester is distributed in only such amount substantially uniformly 35 throughout the fabric plies, they are penetrable substantially instantaneously by a solvent. It is, of course, to be understood that the foregoing stiffener is one cited by way of illustration only, and that I may introduce into various kinds of 40 fabric plies more or less cellulose ester, depending upon the particular class of shoes into which the stiffener is to go. In any event, however, the stiffened fabric plies are preferably sufficiently porous to permit the penetration therewith and therethrough of the solvent in a reasonable period 45 of time, so as to wet substantially all of the surfaces of the preformed cellulose ester film.
- 50 As an example of one special sphere of utility of my invention, I wish to observe that a box toe made up with an adequate number of plies, as hereinbefore described, is highly advantageous in so-called safety shoes. A shoe containing such a box toe has a fore part not only proof against water, perspiration, oil, and other liquids, and 55 high in its dielectric properties, but greatly resistant to heavy shock or impact, and so fits nicely into such hazardous occupations as mining, steel-making, metal pouring, and the like. In these latter connections, I prefer to use cellulose acetate 60 in both the film and as the impregnant for the fabric plies. The cellulose acetate makes for low inflammability in the stiffener as a whole, wherefore, should the shoe fore part come into contact 65 with fire, molten metal, or other heated objects, the wearer's toes are protected against severe 70 burning. I have already adverted to the fact that a shoe stiffener may be constructed, in accordance with my invention, to withstand heavy shock or impact. For instance, a box toe made 75 with seven plies of stiffened fabric and six plies

of film, as illustrated in Figure 3, is so tough and resilient as to withstand, without fracture, pressures of at least about 2500 pounds per square inch. This indicates that a shoe into which such a blank is incorporated offers much resistance at its fore part against heavy impact, and hence minimizes injury to the toes of a wearer when heavy masses accidentally fall upon the fore part. 80

In some instances, the film may consist of nitrocellulose and the outer fabric plies contain cellulose acetate as the stiffening impregnant. In such case, the solvent used for conditioning the blank as a whole for shoemaking should, of course, be one functioning as a solvent or plasticizing agent for both cellulose acetate and nitrocellulose. There are various solvents or solvent mixtures for both these cellulose esters, e. g., acetone, diacetone-alcohol, diethylene glycol acetate, glycol monoacetate, ethylene oxide; and it is not necessary that the solvent or solvent mixture have the same action on both esters. The inflammability of such a shoe stiffener is cut down by the outer plies, which serve to shield the highly combustible nitrocellulose film from direct exposure to heat. Rather than being a cellulose ester, the stiffening agent for the fabric plies may be a compound of another class, capable of undergoing gelatinization by the same solvent designed to act upon the cellulose ester film. For example, I may use an artificial resin, e. g., bakelite varnish, as the stiffening agent for the fabric plies. In such case, the solvent selected for conditioning the stiffener as a whole for shoemaking is one common to both the artificial resin and the cellulose ester film. By using in the fabric plies a stiffening agent whose character is quite different from a cellulose ester, it is possible to realize a combination of characteristics in the composite shoe stiffener unattainable by the use of a single stiffening agent, such as cellulose acetate or nitrocellulose. Thus, the stiffener may comprise fabric plies impregnated with a suitable resin, such as cumar resin, which is characterized by its extreme hardness and stiffness under normal temperature conditions, but which 100 has the fault of being easily shattered by impact. This fault of easy shatterability in the cumar resin carried by the fabric plies may be so offset by the flexibility and resiliency of the cellulose ester film that the stiffener as a unit is characterized by the desirable increase in hardness and stiffness afforded by the cumar resin, while at the same time being adequately resilient and flexible to meet all the needs in service. 110

115 It is preferable that the outer fabric plies in the stiffeners of the present invention be woven or similar textile fabric, so as to contribute mechanical strength to the stiffener. In the case of box toes, such fabric plies are desirable, because the stiffeners undergo considerable pulling stress as they are being formed to the shape of the last. When, however, such a stiffener contains more than three plies, only the outer plies 120 need be made of woven or similar textile fabric. The rest of the fabric plies may be paper felt or similar inexpensive fibrous foundation. 125

Rather than being stiffened by impregnation with a solution of the stiffening agent, the paper felt and/or the woven or other textile fabric plies may be charged with comminuted or powdered stiffening agent. In such instance, high porosity is necessarily a concomitant quality of the stiffened fabric plies. In the case of a paper felt, the cellulose ester or other stiffening agent 130 may be introduced as a powder, precipitate, aque- 135

ous dispersion, or in any other suitably subdivided state into the papermaking pulp in the beater engine before the pulp is formed into a web on the papermaking machine. In the case 5 of a textile fabric, the powdered cellulose ester or other finely divided form of stiffening agent may be forced into the pores and interstices of the fabric in the condition of an aqueous or other suitable paste, by squeeze rolls or their equivalent.

10 I claim:

1. A laminated shoe stiffener, comprising at least three plies bonded together in superposed, face-to-face relationship, the inner ply consisting of a preformed, substantially continuous film of cellulose ester and the outer plies consisting of fabric charged with stiffening agent coming from a source other than said film and capable of being gelatinized by a solvent of said cellulose 15 ester.

2. A laminated shoe stiffener, comprising at least three plies bonded together in superposed, face-to-face relationship, the inner ply consisting of a preformed, substantially continuous film of cellulose acetate and the outer plies consisting of fabric charged with cellulose acetate coming from a source other than said film.

3. A laminated shoe stiffener, comprising a preformed, substantially continuous film of cellulose ester bonded face to face with a fabric impregnated with a stiffening compound other than said cellulose ester but soluble in a solvent of said ester.

4. A laminated shoe stiffener, comprising a preformed, substantially continuous film of nitrocellulose bonded face to face with a fabric impregnated with cellulose acetate.

5. A laminated shoe stiffener, comprising a preformed, substantially continuous film of cellulose ester bonded face to face with a fabric impregnated with a stiffening compound other than a cellulose ester but gelatinizable in a solvent of the ester of said film.

6. A laminated shoe stiffener, comprising a plurality of preformed, substantially continuous films of cellulose ester, bonded face to face in

alternating relationship with fabric plies charged with a stiffening agent coming from a source other than said films and capable of being gelatinized by a solvent of said cellulose ester, said stiffener containing stiffened woven textile fabric as the outer fabric plies and stiffened paper felt as the inner fabric plies.

7. A laminated shoe stiffener especially adapted for use in safety shoes, comprising a plurality of preformed, substantially continuous films of cellulose acetate bonded face to face in alternating relationship with fabric plies charged with cellulose acetate coming from a source other than said films, said stiffener containing as the outer plies woven textile fabric charged with the cellulose acetate.

8. A laminated shoe stiffener, comprising a preformed film of cellulose ester bonded face to face with a fabric charged substantially throughout with stiffening agent in subdivided form and capable of being gelatinized by a solvent of said cellulose ester.

9. A laminated shoe stiffener, comprising a preformed film of cellulose acetate bonded face to face with a fabric charged substantially throughout with cellulose acetate in subdivided form and capable of being penetrated quickly by a cellulose acetate solvent.

10. A laminated shoe stiffener, comprising at least three plies bonded together in superposed, face-to-face relationship, the inner ply consisting of a preformed film of cellulose ester and the outer plies consisting of fabric charged substantially throughout with cellulose ester in subdivided form and capable of being penetrated quickly by a cellulose ester solvent.

11. A laminated shoe stiffener, comprising at least three plies bonded together in superposed, face-to-face relationship, the inner ply consisting of a preformed film of cellulose acetate and the outer plies consisting of fabric charged substantially throughout with cellulose acetate in subdivided form and capable of being penetrated quickly by a cellulose acetate solvent.

STANLEY P. LOVELL. 120

50

125

65

130

60

135

65

140

70

145

150